

## UNITED STATES PATENT OFFICE

2,266,380

## PRETREATMENT OF METAL BEARING SURFACES

George L. Neely and Victor M. Kostainsek, Berkeley, Calif., assignors to Standard Oil Company of California, San Francisco, Calif., a corporation of Delaware

No Drawing. Application May 18, 1940,  
Serial No. 336,008

5 Claims. (Cl. 148—6.5)

This invention relates to pretreated bearing surfaces and to the method of producing the same, particularly to provide a pretreated bearing surface having improved wear-in characteristics and protected from oxidation or rusting. This invention is particularly directed to an improvement over that invention disclosed in the co-pending application of Farrington, et al., entitled "Treatment of metallic frictional surfaces" filed October 19, 1938, Serial No. 235,811.

In the pretreatment of metal bearing or wearing surfaces in order to increase the ability of such surfaces to immediately accommodate high loads without danger of initial failure, processes have now been resorted to of treating such surfaces in order to form on the wear-receiving or bearing surfaces of the ferrous metal bearing elements a sulphide film accompanied with pitting of the surface to produce a multiplicity of lubricant-receiving recesses upon such surfaces. The bearing surfaces when so treated have been found to be extremely susceptible to oxidation or rusting with the result that the said elements produce a very unattractive appearance which is detrimental to the sales of such articles, particularly when it is necessary to retain the materials in stock or to hold the same for a period of time for use or for sale as replacement parts.

It is therefore an object of this invention to provide a method of the pretreatment of metal bearing surfaces in order to increase the ability of such surfaces to take initial loads without failure and which method also provides for the treatment of the said bearing elements to prevent oxidation or rusting of the film or surface so treated.

Another object of this invention is to provide a method of pretreating ferrous metal bearing or wearing surfaces in order to increase the ability of such surfaces to withstand initial extreme pressure loads and which method also includes treatment of such surfaces with a chromate of an alkaline earth metal to prevent oxidation or rusting of the said treated surface or the film produced upon such surface by the said pretreatment.

Another object of this invention is to provide a pretreated metal bearing or wearing element the bearing or wearing surface of which is characterized by having formed thereon or therein an iron sulphide film and further characterized by having its surface pitted and by having upon its surface a coating of an alkali chromate.

Other objects and advantages of our invention it is believed will be apparent from the herein-

after contained detailed description of a preferred embodiment of our invention.

In accordance with our invention, the ferrous metal bearing or wearing member is first treated to enhance its ability to carry initial loads without failure under extreme pressure by reacting the said bearing surface with a chemical reagent capable of reacting with the ferrous metal of the surface to produce an iron sulphide film upon the surface. The reaction of the ferrous metal of the surface and the chemical reagent is preferably carried on under such conditions and for such period of time as will permit the said chemical reagent to selectively etch or pit the surface by selective reaction between the component elements of the surface and the chemical reagent utilized.

Ferrous metal bearing surfaces are usually composed of steel or cast iron or alloys. Chemical reagents which will react with such surfaces to form iron sulphide coatings generally selectively act upon such surfaces particularly with the free ferrite iron in preference to the combined iron or ferrous metal of such a surface with the result that the surface is pitted selectively over the area treated, leaving a multiplicity of fine pits or recesses in the surface. The reaction is also to produce upon the surface and within the pits or recesses formed a deposit or film of iron sulphide. Both the iron sulphide film so produced and the pitting of the surface enhance the ability of the treated surface to carry initial extreme pressure loads without failure. This is as set forth in the co-pending application of Neely, et al., Serial No. 235,542, filed October 17, 1938, for "Pretreated bearing surface and method of producing the same."

In accordance with the method embodying this invention, the pretreated ferrous metal bearing surface is, after the pretreatment, preferably washed or treated to remove any loosely adhering material. The treated surface is next dipped in an alkali chromate solution and allowed to remain in such solution for such period of time as may be required to produce a film or coating of alkali chromate over the bearing surface or the film or coating of iron sulphide previously deposited upon the surface.

We have found that the formation of this alkali chromate coating or film upon the said surface does not decrease or increase the effectiveness of the previous pretreatment but does effectively retard and prevent rusting or oxidation of the surface or the sulphide film or coating previously formed on the surface. Any suitable method

of pretreatment of the bearing surface to produce the iron sulphide film or coating may be resorted to as, for example, any of those methods disclosed in the co-pending applications hereinabove referred to such as the treatment by hydrogen sulphide gas, or active sulphur in any form. The preferred method, however, is to treat the surface in an alkali sulphur bath as, for example, by dipping the ferrous metal surface in a treating solution made up, for example, of 1,000 grams of 47% NaOH solution to which there is added 50 grams of sulphur. The mixture thus produced is heated to a temperature of about 265° F. and stirred until the sulphur is dissolved in the solution and the solution becomes clear. The ferrous metal bearing surface as, for example, any previously machined bearing surface such as a bearing cup, piston rings, cylinder liners, gears, or any other ferrous metal bearing surface, is then immersed in the solution thus prepared for a period of time and at an elevated temperature sufficient to form upon the surface iron sulphide to produce a dual break coating. Any other suitable method of forming the iron sulphide film, however, may be resorted to and of course different concentrations of alkali sulphur solution may be employed and other alkali hydroxides may be substituted for the sodium hydroxide above specified.

Following the formation of the iron sulphide film upon the ferrous metal surface, the surface is washed preferably in warm water to cleanse the same to remove any loosely adhering iron sulphide or other foreign matter from the surface. The cleansed surface as thus produced bearing the iron sulphide coating and which is preferably etched during the process of formation of the coating is then dipped into a solution of alkali chromate ranging anywhere from 1% to 10% alkali chromate to produce upon the surface an alkali chromate film or covering. The particular example of this treatment found suitable is an alkali chromate treating bath which comprises, for example, 1% to 10% of sodium chromate in water.

A surface having this combined treatment has its resistance to rusting or oxidation increased many fold as compared with a surface treated with alkali sulphur solution alone. We have found that this increased resistance to rusting or oxidation may be sufficient to avoid the necessity for application of oil or grease to the surface prior to shipment of the treated ferrous metal machine elements.

Tests of the resistance of such combined treated surfaces to the effects of rusting or oxidation are shown in the following table. In these tests previously machined bearing cups were employed. The tests show, as, for example, Test No. 1, the rusting effect produced upon the treated and untreated surfaces by 15-minute interval sprays upon the surfaces of a 0.2% salt (NaCl) solution where twenty such spray applications were made upon the surfaces.

Test No. 2 differs only from Test No. 1 in the fact that eight such sprays were utilized with the intervals of time between the sprays 1-hour rather than 15-minutes. The extent of the sprays with salt solutions in each case was sufficient to completely cover the surfaces with the

70 salt solution but insufficient to produce dripping or running of the solution off from the surfaces. These tests are:

5 SALT SPRAY TEST 1—(20 sprays of .2% salt solution at 15-minute intervals)

NEW CUPS

|    | Treatment           | Rusting    |
|----|---------------------|------------|
| 10 | None                | Excessive. |
|    | 1% sodium chromate  | Partial.   |
|    | 10% sodium chromate | None.      |

TREATED CUPS

|    | Treatment           | Rusting    |
|----|---------------------|------------|
| 15 | None                | Excessive. |
|    | 1% sodium chromate  | Partial.   |
|    | 10% sodium chromate | None.      |

20 SALT SPRAY TEST 2—(8 sprays of .2% salt solution at 1-hour intervals)

NEW CUPS

|    | Treatment | Rusting    |
|----|-----------|------------|
| 25 | None      | Excessive. |

TREATED CUPS

|    | Treatment          | Rusting    |
|----|--------------------|------------|
| 30 | None               | Excessive. |
|    | 1% sodium chromate | None.      |

Having fully described our invention, it is to be understood that we do not wish to be limited to the details herein set forth, but our invention is of the full scope of the appended claims.

We claim:

1. A method of pretreatment of a bearing surface of ferrous metal, including the steps of pretreating the said surface with an active sulphur reagent to form an iron sulphide film on said surface, and then contacting said surface with an aqueous solution of an alkali chromate.

40 2. A method of pretreatment of a bearing surface of ferrous metal comprising contacting the said surface with an aqueous solution containing an hydroxide of an alkali metal containing dissolved sulphur, washing the surface so treated, and then contacting said surface with an aqueous solution of an alkali chromate.

45 3. A method of pretreatment of a bearing surface of ferrous metal, comprising the pretreatment of said surface with an active sulphur containing chemical reagent to form an iron sulphide film on said surface, and to pit the surface, cleaning the surface so treated of foreign matter, and then contacting said surface with an aqueous solution of an alkali chromate.

50 4. A pretreated bearing surface of ferrous metal characterized in that there is an iron film on said surface, the film consisting of the ferrous metal of the surface and a sulphide radical reacted with an alkali chromate.

55 5. A pretreated bearing surface of ferrous metal characterized in that its bearing area is pitted from the surface and has a film thereon, the film being a reaction product of the ferrous metal of the surface, a sulphide radical, and an alkali chromate.

60 GEORGE L. NEELY.  
VICTOR M. KOSTAINSEK.